

## UNITED STATES PATENT OFFICE

2,011,259

## NONFERROUS ALLOY

William B. Price, Waterbury, Conn., assignor to  
Scovill Manufacturing Company, Waterbury,  
Conn., a corporation of Connecticut

No Drawing. Application December 9, 1931,  
Serial No. 579,985

## 4 Claims. (Cl. 75—1)

This invention relates to an improvement in non-ferrous alloys, and particularly to alloys consisting principally of copper, zinc, aluminum and nickel.

5 I have found that by increasing the zinc content while reducing the copper content and at the same time employing small but essential amounts of nickel and aluminum an alloy is obtained which is harder than alloys of the same metals having less zinc and more copper.

10 A further advantage in manufacturing is that the new alloy is much brighter after annealing than with prior alloys of the same metals having higher percentages of copper and less of zinc. 15 Also, while such prior alloys are very resistant to corrosion under ordinary conditions, yet at the high temperatures of annealing they form a slight scale which necessitates treatment with a pickling solution such as 10% sulphuric acid solution.

20 By reducing the percentage of copper and increasing the percentage of zinc, while maintaining the same ranges of percentages of aluminum and nickel, the new alloy is so bright and free 25 from scale that it is unnecessary to pickle it. A product of this kind is particularly suitable for architectural purposes, especially for exterior sidings or panels.

The alloys of the present invention consist 30 chiefly of copper, zinc, nickel and aluminum, although, of course, in commercial production slight amounts of other metals may be present without injuriously affecting the advantageous properties of the alloy. For example, a slight 35 percentage of lead not exceeding 2% of the whole will be advantageous where the product is to be machined as, for example, by turning.

For a material which is to have a good tensile strength particularly at relatively high temperatures, the most advantageous results are obtained 40 with an alloy consisting chiefly of copper, zinc, nickel and aluminum, in which the relative proportions of the four metals are substantially as follows:

Per cent

|          |    |
|----------|----|
| Copper   | 70 |
| Zinc     | 27 |
| Nickel   | 1  |
| Aluminum | 2  |

An alloy of this composition when extruded into bars and rolled to what is known as 8 numbers hard, gave, on testing, a Brinell hardness number 98. Different samples cut from this strip and annealed at different temperatures, as stated below, gave the following results:

|             |         |         |         |    |
|-------------|---------|---------|---------|----|
| Annealed at | 500° C. | 600° C. | 700° C. |    |
| Brinell No. | 84      | 69      | 38      | 10 |

This is to be compared with prior alloys having the same percentages of nickel and aluminum but with 80% copper and 17% zinc. The latter 15 alloy when formed in the same way and tested after rolling gave a hardness of 95 Brinell and on annealing the samples gave the following results:

|             |         |         |         |    |
|-------------|---------|---------|---------|----|
| Annealed at | 500° C. | 600° C. | 700° C. |    |
| Brinell No. | 70      | 56      | 27      | 20 |

It will be observed that the hardness of the new alloy with more zinc and less copper was higher than that of the prior alloy under each condition specified, and what is particularly significant is the fact that the drop in hardness by 30 annealing at the customary annealing temperature of 500° C. was only 14 numbers Brinell with the new alloy, whereas it was 25 numbers Brinell with the prior alloy having 80% copper.

Other samples of the new alloy of similar composition were made and on analysis showed the following composition:

Copper 70.56, nickel 1.42, aluminum 2.13, zinc by difference 25.89 which, of course, might include a slight amount of impurities.

Comparative tests of this new alloy with the prior alloy of the same metals having copper higher and zinc lower were made for tensile strength, elongation and reduction of area at different temperatures. The prior alloy had the following composition: Copper 80.16%, nickel 1.00%, aluminum 2.07%, zinc, by difference, 16.77%. The results of these comparative tests were as follows:

| Temperature C.          | 25      | 250    | 375    | 500    | 625   | 750   | 875   |
|-------------------------|---------|--------|--------|--------|-------|-------|-------|
| Tensile strengths:      |         |        |        |        |       |       |       |
| New alloy               | 91,600  | 74,100 | 51,900 | 24,900 | 5,100 | 2,700 | 652   |
| Prior alloy             | 100,500 | 89,000 | 50,700 | 16,600 | 7,700 | 4,200 | 2,000 |
| Elongation in 2 inches: |         |        |        |        |       |       |       |
| New alloy               | 16      | 2      | 4      | 40     | 30    | 40    | 37    |
| Prior alloy             | 14      | 4      | —      | —      | 49    | 101   | 142   |
| Reduction of area:      |         |        |        |        |       |       |       |
| New alloy               | 66      | 2      | 5      | 32     | 51    | 40    | —     |
| Prior alloy             | 48      | 12     | 49     | 52     | 89    | 100   | —     |

It will be observed that although the tensile strength of the new alloy at temperatures of 250° and below is somewhat less than that of the prior alloy, yet at temperatures ranging from 375 to 5 500° C. the tensile strength is greater and therefore the new alloy is particularly suitable for use under conditions where it must withstand working stresses at temperatures in the neighborhood of 375° C. to 500° C. This is confirmed also by the 10 figures as to elongation and reduction of area.

In commercial practice the percentage of nickel in the alloy may vary from 1 to 1 1/2% and the aluminum from 2 to 2 1/2% while still retaining the advantages of the invention as to satisfactory 15 tensile strength and hardness of the resulting product under working temperatures as high as 500° C. as, for instance, in equipment for steam plants working at modern high pressures and consequent relatively high temperatures, this result 20 being attained by keeping the percentage of copper below 80% and correspondingly increasing the zinc. It has been found that with nickel and aluminum within the ranges stated hereinabove the copper may vary considerably from the 70% 25 of copper employed in the best embodiment of the invention, provided, however, it be not lower than 60%. At this lower limit of copper, with nickel 1 to 1 1/2, aluminum 2 to 2 1/2 and zinc, including any impurities or slight amounts of other metals, 30 by difference, ranging from 36 to 37, it will be found that the alloy comes through the annealing process in a very bright condition so that where color of this kind is desired, the lower percentage 35 of copper may be employed, but with some reduction in tensile strength as compared with the alloy having 70% copper.

On the other hand, as the percentage of copper is increased from 70% toward 80%, the color is not quite so bright after annealing, the tensile 40 strength at temperatures around 375° to 500° C. is not as high as that of the 70% alloy, and the hardness is less than that of said 70% alloy, but at temperatures below 375° C. the tensile strength is relatively higher. Therefore, to attain the 45 advantages of the present invention the copper should be kept within the range of 60 to about 80% of the total of the four metals, copper, zinc, nickel and aluminum, and any impurities or additional metals should be kept below 1 1/4%. Hence, 50 the zinc should not be less than 16 1/4% and not more than 38% of the complete alloy, the lower figure allowing for the impurities or other metals such as some lead. In the best embodiment of the invention, as hereinbefore set forth, the impurities should be reduced to a minimum, for example, so as to total not more than half of one percent of 55 the total alloy.

Although as pointed out above, the alloy consists chiefly of copper, zinc, nickel and aluminum, and the proportions may range as stated, viz: copper 60-79, zinc, about 38 to 16 1/4%, aluminum 60 1 to 2 1/2%, nickel 1 to 2 1/2%, yet to obtain the best balance of the properties for commercial purposes, viz: good tensile strength, hardness and freedom from scale after annealing, it is well to 65 keep closer to the ideal formula employing 70% copper, 1 to 2 1/2% aluminum, 1 to 2 1/2% nickel and the balance substantially all zinc, except for impurities which, if present, should not exceed 70 1/2%.

Where, however, the material is to be used for

exposed architectural purposes, and a durable golden color is demanded while the tensile strength need not be so high, the ideal composition for such purpose will have copper about 60 to 65 percent, aluminum 1 to 2 1/2%, nickel 1 to 2 1/2%, impurities, including lead, not to exceed 1/2% and the balance zinc.

In practice it is sufficient to maintain the nickel and aluminum within the ranges stated and to maintain the copper within a range of about 5% each side of the ideal, that is to say within the range of 65% to 75%, the zinc constituting substantially all of the remainder, that is, about 20 to 33 percent of the whole. If there are any impurities or other metals such as lead, they should not exceed one percent, and the percentage of zinc should be reduced an equivalent amount.

An alloy embodying the present invention has all the advantages of the previously known high copper alloys consisting chiefly of copper, zinc, 20 nickel and aluminum in regard to corrosion resistance, lack of tendency to season crack and ease of extrusion into rods or tubes at relatively low temperatures and relatively low pressures. It has a tensile strength nearly as high at low temperatures, say from 25° C. to 250° C. and is much improved as to tensile strength in the range of 375 to 500° C. Its hardness is also higher at all temperatures.

What is claimed is:

1. An alloy consisting essentially of copper, aluminum, nickel and zinc, in proportions substantially as follows:

|                                    | Per cent   |
|------------------------------------|------------|
| Copper                             | 60 to 75   |
| Aluminum                           | 1 to 2 1/2 |
| Nickel                             | 1 to 2 1/2 |
| Balance zinc except for impurities |            |

2. An alloy consisting essentially of copper, aluminum, nickel and zinc, in proportions substantially as follows:

|                                    | Per cent   |
|------------------------------------|------------|
| Copper                             | 70         |
| Aluminum                           | 1 to 2 1/2 |
| Nickel                             | 1 to 2 1/2 |
| Balance zinc except for impurities |            |

3. An alloy having the following composition:

|                                     | Per cent     |
|-------------------------------------|--------------|
| Copper                              | 60 to 75     |
| Aluminum                            | 1 to 2 1/2   |
| Nickel                              | 1 to 2 1/2   |
| Lead                                | 1/2 to 1 1/4 |
| Balance zinc, except for impurities |              |

4. An alloy having the characteristics of good tensile strength falling only slowly at increasing temperatures up to 500° C.; capability of taking a relatively high hardness falling off only slowly up to 500° C.; good resistance to corrosion under ordinary conditions, and very small scale formation after annealing, said alloy having the following composition:

|                                                                  | Per cent   |
|------------------------------------------------------------------|------------|
| Copper                                                           | 60 to 70   |
| Aluminum                                                         | 1 to 2 1/2 |
| Nickel                                                           | 1 to 2 1/2 |
| Lead, to modify machinability                                    | 0 to 1 1/4 |
| Zinc constituting the remainder, except for traces of impurities |            |

WILLIAM B. PRICE.